

## UNITED STATES PATENT OFFICE

2,651,587

## TREATMENT OF TEXTILE MATERIALS

Elmer H. Rossin, Melrose, Mass., assignor to Monsanto Chemical Company, St. Louis, Mo., a corporation of Delaware

No Drawing. Application June 3, 1947,  
Serial No. 751,995

10 Claims. (Cl. 117—138.8)

1

This invention relates to the sizing of nylon warp yarns and threads for the purpose of improving their weaving characteristics.

It has been common practice to apply starch size solutions to the warp yarn prior to weaving for the purpose of increasing the strength of the yarn, reducing shedding during passage through the loom or for other reasons. However, ordinary starch sizes on drying have the disadvantage of dusting to a considerable extent both in the slasher and in the loom. Moreover, they do not reduce shedding as much as might be desired. Other sizes for nylon yarns that have been used include polyvinyl alcohol, protein sizes and modified starches, but when such sizes are employed, excessive dusting in the loom is found as well as an excessive number of breaks in the warp yarns.

It is a primary object of the present invention to provide sizing or slashing formulations, which result in a markedly decreased amount of dusting and shedding and at the same time produce yarns of enhanced strength and resistance to breakage in the loom.

A further object of the invention is to provide a relatively permanent sizing solution which can be applied to the yarn at room temperature if desired without gelling or otherwise becoming unfit for use.

Still further objects of the invention will become apparent from the following detailed description and appended claims.

In accomplishing the above objects the warp yarn or thread is treated, as for example in the size box of the conventional slasher, with an aqueous solution or dispersion of an ammonium, quaternary ammonium, sodium, potassium or other alkali salt of the copolymer of styrene and an alkyl ester of maleic acid, after which the yarn is dried over dry cans or by any other suitable method including air drying at room temperature. The alkyl esters which may be used to make the copolymer include those in which the alkyl group contains from 1 to 4 carbon atoms, including the methyl, ethyl, propyl, butyl and secondary butyl esters of maleic acid. The concentration of the styrene-maleic ester salt in the bath and the pick-up of the size box rolls should be adjusted to deposit on the yarn from 2 to 12% by weight of the salt on the weight of the yarn, but preferably between about 4 and 7%. Although good results may be obtained in some instances, as when a heavy yarn is treated, by using the bath at room temperatures, it is usually desirable to have the bath or solution at somewhat elevated temperatures, usually between about

2

120 and 150° F., to insure uniform penetration. In the event that a semipermanent finish is desired on the warp threads, it is necessary, when ammonium salts are used, to dry the warp yarns, or the fabric prepared therefrom, at a sufficiently elevated temperature to set the resin. Under such circumstances, the yarn is heated preferably at 250 to 300° F. during drying, but satisfactory results may be obtained at temperatures as low as 200° F. When sodium or potassium salts are used, however, it is not essential to dry at elevated temperatures, but when a semi-permanent finish is desired, the yarns, or the fabric prepared therefrom, must be subjected to a dilute acid finishing bath in order to set the resin on the yarn or fabric.

The copolymer of styrene and esters of maleic acid used in accordance with this invention is a well-established product which may be prepared in several ways. One of the well-known methods is mass polymerization, which involves heating styrene and an ester of maleic acid at temperatures between about 100 and 300° F. for several hours or more using for each mol of styrene varying amounts of the ester of maleic acid, for example between 0.25 and 4 mols, but preferably in the neighborhood of equimolecular quantities. Preferably, the materials are heated cautiously, as in a water bath. Another method which may be used is known as the solvent process which involves reacting the styrene and the esters of maleic acid at slightly elevated temperatures in the presence of a solvent which is capable of dissolving both the starting materials and the finished polymer, such as acetone. If desired, the copolymerization may be carried out in the presence of a catalyst, such as benzoyl peroxide.

Another method which may be used to prepare the copolymer of styrene and the alkyl ester of maleic acid involves copolymerizing styrene and maleic anhydride by any of the standard procedures described above, after which the copolymer is reacted in alcohol by the regular chemical procedure for alcoholysis, thereby producing the ester of the copolymer. It is also possible, but not preferred, to mix simultaneously the styrene-maleic anhydride and alcohol and then polymerize the mixture by any of the standard procedures.

50 A further understanding of the invention will be obtained from the following examples, the parts being given by weight:

## Example I

55 A solution of an ammonium salt of styrene-maleic acid ester resin was prepared by mixing

together 150 parts of the secondary butyl ester of styrene-maleic acid, prepared by copolymerizing equimolecular quantities of styrene and the secondary butyl ester of maleic acid at about 200° F. in a water bath, 100 parts of 26% NH<sub>4</sub>OH and 1750 parts of water. The resulting mixture was then heated from 200 to 212° F. with stirring, and maintained at this temperature until a uniform, somewhat viscous transparent solution resulted. This required about one hour. The resulting size was then poured in the size box of a 5 can silk slasher, after which a warp of 200/34/5Z nylon yarn was passed at a speed of 15 yards per minute through the size solution, which was maintained at 150° F., and dried on the dry cans at 180° F. By proceeding in this way, excellent weaving was obtained and the resulting fabric was substantially free of floats. The size was easily removed from the finished fabric by washing with warm water.

*Example II*

A 7% solution of the sodium salt of the styrene-maleic acid ethyl ester was prepared by mixing together 140 parts of the ethyl ester of styrene-maleic acid, prepared by copolymerizing equimolecular quantities of styrene and the ethyl ester of maleic acid at about 200° F. in a water bath, 60 parts of 50% NaOH and 1800 parts of water. The resulting mixture was then heated from 200 to 212° F. with stirring, and maintained at this temperature until a uniform, somewhat viscous transparent solution resulted, which required about one hour. After cooling the resulting solution to 125° F., it was poured into the size box of a 7 can Johnson slasher, after which a warp of 200/34/5Z nylon was passed through the solution and dried on the dry cans in the usual manner. The treated yarn was then rolled up on a beam and woven. As a result of treating the yarn in the above manner prior to weaving, numerous improvements were noted in the weaving process and in the resulting fabric, including a smaller number of broken ends, fewer broken filaments, and a final fabric which is smoother and more uniform than fabrics woven in the customary way. The size was easily removed from the finished fabric by washing with warm water.

*Example III*

A solution of an ammonium salt of styrene-maleic acid ester resin was prepared as described in Example I. The resulting size solution was then poured in the size box of a 5 can silk slasher, after which a warp of 200/34/5Z nylon yarn was passed at a speed of 15 yards per minute through the size solution, which was maintained at 150° F., and dried on the dry cans at 180° F. As a result of the above treatment, the weaving of the yarn was greatly facilitated and the resulting fabric was substantially free of floats. The fabric was further heated on a tenter frame at 275° F., which produced a semi-permanent somewhat stiffened finish.

By treating nylon warp yarns with the sizing agents described herein, it is possible to carry out the weaving with a minimum amount of dusting and shedding and with the atmosphere of the room at relatively low humidities. The treated yarn is exceptionally strong and pliable and resistant to abrasion with the result that the number of breaks occurring during weaving is reduced to a minimum. Moreover, the fabric prepared from yarn sized in accordance with the

present invention has a semi-permanent, generally stiffened finish without further treatment, but if desired, it may be subjected to additional finishing operations. When goods are sized in the conventional manner with starches, gums or the like, it is necessary to desize before dyeing or finishing, as these commonly used sizes retard or interfere with the absorption of dyestuffs or finishing agents. When salts of styrene-maleic ester resin are employed however, particularly the ammonium salts, it is possible to eliminate the expensive and cumbersome step of desizing and to dye and finish the fabric evenly and uniformly.

In some cases it is advantageous to add small amounts of softening agents to the size bath, including such materials as sulfonated oils, soaps, emulsified tallow, emulsified oils, glycerine and the like.

It is customary to apply the sizing materials described herein to yarns. However, it is possible to obtain similar results by treating fibers, either initially or at any stage of their processing prior to spinning, after which the fibers may be spun to obtain yarns of the desired weaving characteristics. Fabrics prepared from such yarns also have the desired semi-permanent finish hereinbefore mentioned.

Where reference is made in the appended claims to aqueous solutions, it is to be understood that this is intended to include aqueous dispersions, as it is believed where ammonium salts are employed, the salt is actually present in the form of a colloidal dispersion.

What is claimed is:

1. The method of sizing nylon warp yarns which comprises treating said yarns with a composition consisting essentially of an aqueous solution of a salt of the copolymer of a substance selected from the group consisting of styrene and substituted styrenes and an alkyl ester of maleic acid, in which the alkyl group contains from 1 to 4 carbon atoms, said salt being selected from the group consisting of sodium and potassium salts, and then drying said yarns.

2. The method of sizing nylon warp yarns which comprises treating said yarns with a composition consisting essentially of an aqueous solution of a salt of the copolymer of styrene and an alkyl ester of maleic acid, in which the alkyl group contains from 1 to 4 carbon atoms, said salt being selected from the group consisting of sodium and potassium salts, and then drying the yarns.

3. The method of sizing a nylon warp yarn which comprises treating said yarn with a composition consisting essentially of an aqueous solution of a salt of the copolymer of styrene and an alkyl ester of maleic acid, in which the alkyl group contains from 1 to 4 carbon atoms, said salt being selected from the group consisting of sodium and potassium salts and being deposited on said yarn in amounts varying from 2 to 12% by weight, and then drying said yarn.

4. A nylon warp yarn impregnated with a salt of the copolymer of styrene and an alkyl ester of maleic acid, in which the alkyl group contains from 1 to 4 carbon atoms, said salt being selected from the group consisting of sodium and potassium salts.

5. A woven nylon fabric containing nylon warp yarns which are impregnated with a salt of the copolymer of styrene and an alkyl ester of maleic acid, in which the alkyl group contains from 1 to 4 carbon atoms, said salt being selected from

the group consisting of sodium and potassium salts.

6. The method of sizing nylon warp yarns which comprises treating said yarns with a composition consisting essentially of an aqueous solution of the sodium salt of the copolymer of styrene and an alkyl ester of maleic acid, in which the alkyl group contains from 1 to 4 carbon atoms, and then drying the yarns.

7. The method of sizing a nylon warp yarn which comprises treating said yarn with a composition consisting essentially of an aqueous solution of a sodium salt of the copolymer of styrene and the secondary butyl ester of maleic acid, said salt being deposited on said yarn in amounts varying from 2 to 12% by weight, and then drying said yarn.

8. The method of sizing a nylon warp yarn which comprises treating said yarn with a composition consisting essentially of an aqueous solution of a sodium salt of the copolymer of styrene and the ethyl ester of maleic acid, said salt being deposited on said yarn in amounts varying from 2 to 12% by weight, and then drying said yarn.

9. The method of sizing a nylon warp yarn which comprises treating said yarn with a composition consisting essentially of an aqueous solution of a sodium salt of the copolymer of styrene and

the methyl ester of maleic acid, said salt being deposited on said yarn in amounts varying from 2 to 12% by weight, and then drying said yarn.

10. The method of sizing a nylon warp yarn which comprises treating said yarn with a composition consisting essentially of an aqueous solution of a sodium salt of the copolymer of styrene and a propyl ester of maleic acid, said salt being deposited on said yarn in amounts varying from 2 to 12% by weight, and then drying said yarn.

ELMER H. ROSSIN.

References Cited in the file of this patent

UNITED STATES PATENTS

| Number    | Name                    | Date          |
|-----------|-------------------------|---------------|
| 1,976,679 | Fikentscher et al. .... | Oct. 9, 1934  |
| 2,047,398 | Voss et al. ....        | July 14, 1936 |
| 2,300,566 | Hahn et al. ....        | Nov. 3, 1942  |
| 2,324,601 | Spanagel ....           | July 20, 1943 |
| 2,324,739 | Stoops et al. ....      | July 20, 1943 |
| 2,402,625 | Martin ....             | June 25, 1946 |
| 2,469,407 | Powers et al. ....      | May 10, 1949  |
| 2,469,408 | Powers et al. ....      | May 10, 1949  |
| 2,469,409 | Powers et al. ....      | May 10, 1949  |
| 2,537,018 | Barrett ....            | Jan. 9, 1951  |
| 2,586,477 | Niles ....              | Feb. 19, 1952 |